

Aug. 5, 1969

R. THOMAS ET AL

3,458,901

DEVICE FOR SPINNING VISCOSE

Filed Aug. 1, 1966



INVENTORS

Rainer Thomas,  
Wilfried Keiller and  
Paul Heber

by Michael S. Stricker  
Attorney

## 1

3,458,901

### DEVICE FOR SPINNING VISCOSE

Rainer Thomas, Wilfred Keiler, and Paul Weber, Siegburg, Germany, assignors to Phrix-Werke Aktiengesellschaft, Hamburg, Germany

Filed Aug. 1, 1966, Ser. No. 569,382

Claims priority, application Germany, Aug. 19, 1965,  
P 37,483

Int. Cl. D01d 5/06

U.S. Cl. 18—8

6 Claims 10

### ABSTRACT OF THE DISCLOSURE

Regenerated cellulose is spun by extruding viscose into a formaldehyde-containing precipitating bath so as to form a rope of coagulated filaments, the thus-formed rope is passed downwardly through a steaming zone in which the rope is contacted with steam having a temperature between 95 and 110° C., and from there directly through a watering zone in which the steamed rope is contacted from all sides with hot water having a temperature between about 70 and 95° C., and the rope is stretched during the steaming and watering thereof to between about 300% and 500% of its original length. 15 20 25

The present invention relates to device for spinning viscose and, more particularly, the present invention is concerned with producing fibers, filaments, threads and 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000

It is known to use formaldehyde for stabilizing by methylolation, the cellulose xanthogenic acid which is formed by spinning viscose into an acidic, zinc-free spinning bath. By using highly substituted cellulose xanthogenates having gamma values higher than 80, it is possible in this manner to obtain threads which can be stretched in hot baths by between 300 and 500% and which possess great strength and extremely low extensibility. The methylolation will cause an improvement in the extensibility of the threads, however it will also cause several different problems during the regeneration of the cellulose.

The degree of substitution of the cellulose after stretching is considerably higher than if the spinning is carried out in the absence of formaldehyde. If one does not cause substantial splitting off of the residual xanthate groups while the spinning rope is still under tension, regeneration will take place only after cutting the rope or after spinning the endless filaments in a centrifuge, i.e., in untensioned condition. The decomposition of the residual xanthate in untensioned condition will cause a reduction in the orientation of the cellulose crystallites, which orientation had been caused previously by the stretching of the fiber, and this reduction of orientation will reduce the strength of the fibers and threads. Furthermore, fibers with an excessive residual substitution during decomposition in tensioned condition tend to form adhesions of the single capillaries into clogged fibers of relatively high titre.

Thus, the requirements made on the bath in which the stretching of the spun fibers is carried out are somewhat contradictory and difficult to comply with. On the one

## 2

hand, the degree of decomposition of the xanthate should be low in order to permit maximum stretching of the rope, on the other hand, after the stretching, the xanthate should be decomposed as completely as possible while the rope is still under tension.

It is therefore an object of the present invention to overcome the above-discussed difficulties and disadvantages connected with spinning and subsequent stretching of regenerated cellulose with utilization of a formaldehyde-containing spinning bath.

It is another object of the present invention to provide a method and device which will permit stretching of the yarn combined with decomposition of the xanthate while the yarn is still in tensioned condition, and which will permit carrying out the process in a simple and economical manner.

Other objects and advantages of the present invention will become apparent from a further reading of the description and of the appended claims.

With the above and other objects in view, the present invention contemplates in a spinning arrangement adapted for spinning regenerated cellulose, in combination, spinning means for spinning a yarn, bath means for immersing the yarn in a hot liquid, guide means for guiding the yarn along a predetermined path from the spinning means to the bath means and through the latter, and steaming means along the path between the spinning means and the bath means for steaming the yarn during its passage therethrough.

It is also within the scope of the present invention to provide in a method of producing spun bodies of regenerated cellulose, the steps of spinning viscose into a formaldehyde-containing precipitating bath so as to form a coagulated rope, contacting the thus formed coagulated rope first with steam having a temperature of between about 95 and 110° C., and thereafter with hot water of between about 70 and 95° C., and stretching the rope, while the same is contacted by the steam and water, by between about 300 and 500% of its original length.

The present invention permits in a simple and effective manner to obtain maximum stretching of the rope combined with decomposition of the xanthates while the rope is still under tension.

The coagulated threads may be stretched in steam preferably having a temperature between about 95 and 110° C., and in water preferably having a temperature of between 70 and 95° C. Stretching preferably may be by between 300 and 500% of the original length of the thread. Thereby it is preferred to pass the threads from contact with steam directly into contact with the hot water bath.

The provision of a short steaming device preceding the hot water bath will assure a favorable sequence of stretching and decomposition of the rope. Preferably, steaming and hot water bath follow each other immediately so that the rope leaving the steam atmosphere is directly introduced into the hot water whereby the zone in which predominantly stretching and the zone in which predominantly decomposition takes place will be determined by the deformability or plasticity of the rope. Due to the fact that the zones of predominantly stretching of the rope and of decomposition of the same change over into each other and partly overlap it is primarily the deformability of the rope which determines the zone in

which predominantly stretching is carried out. This direct and uninterrupted sequence of steaming and hot water treatment is therefore preferable to a treatment in which there is a clear separation between stretching and decomposition of the rope, for instance as would be the case by interposition of a withdrawal means between the steaming zone and the hot water bath.

The method of the present invention gives particularly good results in connection with conventional spinning methods according to which threads of unripened viscose containing between 4 and 7% cellulose, having an alkali factor of between 1.0 and 1.4 and a gamma value greater than 70 are spun into a cold, heavy metal salt-free spinning bath containing per liter between 60 and 90 grams sulfuric acid, between 1.5 and 15 grams formaldehyde, and between 100 and 150 grams sodium sulfate. Particularly good results are obtained by maintaining the cellulose content of the unripened viscose at between 4.5 and 5.5, the alkali factor at between 1.25 and 1.35 and the gamma value higher than 80, and by maintaining the spinning bath at a temperature of between 23 and 27° C., whereby the spinning bath preferably will contain per liter between 68 and 72 grams of sulfuric acid, between 10 and 17 grams formaldehyde and between 130 and 140 grams of sodium sulfate.

The results achieved by following the method of the present invention, including the stretching of the rope in steam and hot water as well as the decomposition of the xanthogenates will be described in an example further below and by the analytical results given in Tables I and II with respect to the rope after treating of the same in various stretching devices and prior to stretching.

Prior to introduction into the steam tube, D, the rope contains considerable proportions of formaldehyde and sulfuric acid. The degree of substitution is high.

After passage through the steam tube, C, in which the rope is completely stretched, formaldehyde content and acid content are still high and the degree of substitution has dropped to only 55% of its original value.

The formaldehyde and acid content will stabilize the methylolated cellulose xanthogenic acid during stretching in steam of for instance 99° C.

Since saturated steam is preferably used, the actual temperature of the steam will depend on barometric pressure and may be as low as about 95° C. However, it is also possible to use somewhat superheated steam up to a temperature of about 110° C. Thus, generally, the steaming with simultaneous stretching of the rope will be carried out at a steam temperature of between about 95 and 110° C.

If the rope is continually decomposed after the steam treatment and in untensioned condition, the previously high degree of orientation of the cellulose molecules will be reduced and thus the quality of the rope and yarn will be impaired.

By stretching in a hot water bath, for instance of 87° C. and containing 3.9 grams per liter of sulfuric acid and 1.5 grams per liter of formaldehyde, without a preceding steaming of the rope, different results will be obtained as indicated at B.

The formaldehyde content of the rope will be greatly reduced, the greater portion of the acid will be washed out and the decomposition of the methylolated cellulose xanthogenic acid will proceed to a considerable extent. Thus, under these conditions, the stabilizing effect of formaldehyde and acid is not achieved and the decomposing effect will dominate. For this reason, it is not possible to accomplish in a hot water bath alone stretching to such a high degree as can be achieved by stretching the rope in a combination of steam and hot water treatment, or by steam treatment alone, since the decomposition of the methylolated cellulose and xanthogenic acid proceeds much faster in the hot water bath than in the steam tube. The quality of the thus obtained fibers is not as good

as that obtained by the inventive combination of steam and hot water treatment.

By proceeding in accordance with the present invention, i.e., by combining steam treatment and hot water treatment during stretching and tensioning of the rope, complete decomposition of the cellulose xanthogenic acid will be achieved (A). A better fiber quality is obtained which is superior to that obtained by either using steam treatment alone or hot water treatment alone.

Furthermore, by stretching the rope in contact with steam, the major portion of the hydrogen sulfide content of the rope will be expelled. Thus, the undesirable interaction between hydrogen sulfide and formaldehyde which may lead to water insoluble polymers of thioformaldehyde will not take place during hot water treatment and thereby the content of the rope on water insoluble sulfur compounds will be lower than that achieved by using only the hot water bath and omitting the steam treatment.

A device for carrying out the process of the present invention preferably includes a steam tube formed of a material which is resistant against acid, formaldehyde and temperatures of up to 110° C., which tube is arranged between the top godet and a hot water bath. Preferably, the steam tube extends downwardly from the top godet to the hot water bath in vertical direction. If the lower end of the steam tube is immersed in the hot water bath, a hydraulically closed system is obtained and it is assured that the rope will enter the hot water bath directly from the steaming zone.

Furthermore, preferably a direction changing means or roller is located in the hot water bath, which roller or the like, or other guide means, is not driven, so that between the first godet of the spinning device and the final withdrawal means the stretching is carried out in a stepless, continuous manner throughout the steaming and hot water zone. It is achieved thereby that more than 90% of the total stretching of the rope will take place in the steam tube which, as pointed out above, preferably is fed with saturated or low pressure steam, and the hot water bath will serve predominantly for decomposing the xanthate groups of the rope.

The novel features which are considered as characteristic for the invention are set forth in particular in the appended claims. The invention itself, however, both as to its construction and its method of operation, together with additional objects and advantages thereof, will be best understood from the following description of specific embodiments when read in connection with the accompanying drawing, in which the figure shows a schematic elevational view of a spinning device or arrangement in accordance with the present invention.

Referring now to the drawing, it will be seen that between the top godet 2 of the spinning device and hot water bath 5 a tube 3 is arranged communicating with steam conduit 4, and the rope is passed through tube 3. For facilitating the initial operation of the device, the steam tube 3 preferably extends vertically between top godet 2 and hot water bath 5, so that the rope can initially be passed under the force of gravity downwardly through steam tube 3. After passing through steam tube 3, the rope is guided by non-driven direction changing roller 6 through hot water bath 5, and withdrawn by means of a final conventional withdrawal arrangement 7.

The invention will now be further described in the following example, with reference to the drawing, however, without limiting the invention to the specific details of the example.

#### EXAMPLE

Viscose containing 5.14% cellulose, and 6.47% sodium hydroxide which had been produced with 64.3% carbon disulfide, is spun at a gamma value of 88.0 and a viscosity of 113 seconds (dropping ball method), through a nozzle containing 3,600 openings of 60 microns diameter. The viscose is spun into an aqueous precipitating

bath 10 maintained at a temperature of 24° C. and containing per liter 73.2 grams H<sub>2</sub>SO<sub>4</sub>, 129 grams Na<sub>2</sub>SO<sub>4</sub>, and 11.8 grams formaldehyde.

The filament is immersed in the bath for a length of 12 centimeters. The thus formed rope of 3,600 individual filaments is withdrawn from the bath by means of a first godet 11, at a speed of 7 meters per minute, and passed over the top godet which rotates at 13 meters per minute. From thereon the cable passes through a vertically arranged glass tube fed with low pressure steam of 99° C. and having an inner diameter of 30 mm. and a length of 800 mm. The lower end portion of the glass tube is immersed for a depth of 20 mm. into the hot water bath 5, the latter containing 3.9 grams per liter sulfuric acid and 1.5 grams per liter formaldehyde. In this manner the rope passes immediately from the steaming zone 3 into the hot water bath 5 maintained at 87° C., and in bath 5 the direction of the rope is changed by guide roller 6 by 90 degrees. The rope passes through bath 5 for a length of 300 mm. The rope is then passed to a conventional final withdrawal means 7 which turns at a speed of 34.3 meters per minute.

The thus obtained rope was then cut in conventional manner into staple fibers of 40 mm. length and, without being desulfurized, decomposed in water of 79° C. and containing 2 grams of sulfuric acid per liter, and thereafter bleached, further treated in conventional manner and dried. The thus obtained staple fibers were free of clogged fibers.

Staple fibers were also produced under similar conditions however passage through the steam tube was eliminated and thus the rope was stretched and decomposed only in hot water bath 5 having the composition and temperature described above. Stretching was carried out by 350%. Again, the staple fibers were free of clogged single capillaries.

Again, under the same general operating conditions, staple fibers were produced by proceeding as described above, with passage of the rope through the steam tube but eliminating the subsequent hot water bath. Stretching was carried out by 390%. The thus obtained staple fibers did include clogged single capillaries.

Table I below gives the results of analytical determinations carried out with ropes which were produced according to the present invention by passing the rope under tension through the steam tube and the hot water bath 5. The analytical results obtained with the rope produced according to the present invention are described under A.

Corresponding analytical results for a rope which was stretched only in hot water and produced without passage through the steam tube are indicated under B and analytical results of ropes produced by passage through the steam tube but under elimination of the subsequent water bath are indicated under C. For purpose of comparison there are given also the analytical results obtained with a rope prior to being stretched and these results are indicated under D.

TABLE I

| Stretching method | Composition of rope stretched as indicated (in percent by weight of cellulose content) |                          |              |                  |                                |
|-------------------|----------------------------------------------------------------------------------------|--------------------------|--------------|------------------|--------------------------------|
|                   | Total CS <sub>2</sub>                                                                  | Xanthate CS <sub>2</sub> | Formaldehyde | H <sub>2</sub> S | H <sub>2</sub> SO <sub>4</sub> |
| A-----            | 9.14                                                                                   | 3.73                     | 2.78         | 0.039            | 0.03                           |
| B-----            | 12.8                                                                                   | 6.35                     | 3.91         | 0.046            | 0.01                           |
| C-----            | 28.2                                                                                   | 17.1                     | 11.60        | 0.113            | 8.75                           |
| D-----            | 43.1                                                                                   | 31.4                     | 15.05        | 0.566            | 18.40                          |

Table II below describes the characteristics of the completed fibers and again A denotes stretching in accordance with the present invention, B stretching in hot water only, and C stretching in the steam tube without subsequent hot water treatment. The higher quality of the fibers produced in accordance with the present invention is immediately apparent.

TABLE II

| Stretching Method | Fiber characteristics |                        |              |                              |                     |     |
|-------------------|-----------------------|------------------------|--------------|------------------------------|---------------------|-----|
|                   | Individual denier     | Sulfur content percent | Strength Rkm | Breaking elongation, percent | Tenacity (loop) Rkm |     |
| A-----            | 1.21                  | 0.005                  | 47.8 36.7    | 7.8 7.9                      |                     | 9.2 |
| B-----            | 1.37                  | 0.03                   | 39.2 28.7    | 10.7 11.5                    |                     | 7.6 |
| C-----            | 1.31                  | 0.008                  | 42.1 31.9    | 11.2 11.6                    |                     | 7.8 |

The abbreviation "cond." is meant to denote that the fiber has been conditioned by being kept prior to testing for 24 hours at 22° C. and 65% relative humidity.

The abbreviation "Rkm" denotes the "kilometric length," i.e., the length of the fiber of the same type which must be suspended from the fiber to be tested in order to break the latter.

It will be understood that each of the elements described above, or two or more together, may also find a useful application in other types of spinning arrangements differing from the types described above.

While the invention has been illustrated and described as embodied in a spinning arrangement adapted for spinning regenerated cellulose, it is not intended to be limited to the details shown, since various modifications and structural changes may be made without departing in any way from the spirit of the present invention.

Without further analysis, the foregoing will so fully reveal the gist of the present invention that others can by applying current knowledge readily adapt it for various applications without omitting features that, from the standpoint of prior art, fairly constitute essential characteristics of the generic or specific aspects of this invention and, therefore, such adaptations should and are intended to be comprehended within the meaning and range of equivalence of the following claims.

What is claimed as new and desired to be secured by Letters Patent is:

1. An arrangement for spinning regenerated cellulose, comprising, in combination, spinning means for spinning viscose, said spinning means including a viscose-precipitating bath, and spinning nozzle means located in said bath for extruding viscose solution into the same so as to form filaments; steaming means operatively associated with said spinning means for contacting the thus formed filaments with steam, said steaming means comprising at least one upright tube having an inlet for said filaments at its upper end and an outlet therefor at its lower end; watering means including an elongated vessel arranged underneath said at least one upright tube for substantially freely moving said filaments therethrough, said vessel being capable of being filled with hot water up to a predetermined level and said at least one upright tube extending downwardly into said vessel with said outlet of said tube being located below said predetermined level and closer to one end of said elongated vessel, so that filaments moving downwardly through said tube and passing through said outlet will be directly introduced into said vessel below said predetermined level; and guide means for moving filaments, in the indicated sequence, from said precipitating bath through said tube and said vessel, said guide means including driven draw roller means located in said vessel in the direction of movement of said filaments downstream of the other end of said vessel.
2. An arrangement as defined in claim 1, and including steam supplying means for introducing steam into said upright tube.

3. A spinning arrangement as defined in claim 2, wherein said steam supply means include conduit means communicating with said tube intermediate said opposite ends thereof.
4. A spinning arrangement as defined in claim 1, wherein said tube extends in substantially vertical direction.

5. A spinning arrangement as defined in claim 1, wherein said elongated tube consists of a material resistant to acid, formaldehyde and temperature up to 110° C.

6. An arrangement as defined in claim 1, wherein said guide means include non-driven direction changing means located in said vessel for changing the direction of movement of said filaments therein.

|           |         |                      |           |
|-----------|---------|----------------------|-----------|
| 2,984,889 | 5/1961  | Braunlich et al. --- | 264—197 X |
| 3,109,698 | 11/1963 | Klein et al. -----   | 264—197 X |
| 3,140,957 | 7/1964  | Tanabe et al. -----  | 264—290 X |
| 3,351,696 | 11/1967 | Drisch -----         | 264—197 X |
| 3,352,957 | 11/1967 | Drisch -----         | 264—197 X |

## FOREIGN PATENTS

236,029 9/1964 Austria.

## References Cited

## UNITED STATES PATENTS

|           |         |                      |           |
|-----------|---------|----------------------|-----------|
| 2,317,152 | 4/1943  | Costa et al. -----   | 264—196 X |
| 2,392,582 | 1/1946  | Kadt -----           | 264—202   |
| 2,488,665 | 11/1949 | Heim -----           | 264—188   |
| 2,692,875 | 10/1954 | Weinstock et al. --- | 28—629 X  |

10 DONALD J. ARNOLD, Primary Examiner

J. H. WOO, Assistant Examiner

U.S. CL. X.R.

264—188, 197